

Patented Jan. 18, 1927.

1,614,820

# UNITED STATES PATENT OFFICE.

ADOLF BECK, OF BITTERFELD, GERMANY.

## MAKING CASTING MOLDS.

No Drawing. Original application filed May 25, 1922. Serial No. 583,717, and in Germany September 4, 1922. Divided and this application filed July 22, 1925. Serial No. 45,420.

My invention refers to the preparation of molds for the melting and casting of easily oxidizable metals such as magnesium and its alloys. It is an object of my invention to provide means whereby the oxidizing action of steam on castings of such metals is prevented, especially as regards castings made in sand molds.

As is well known to those skilled in the art, if it is intended to cast metals, such as magnesium and its alloys, which are liable to get oxidized in heated condition, the casting being effected with the aid of the sand molds hitherto generally employed, such molds must be carefully dried, in order to obtain good castings. If the molds are not dried carefully, a reaction will take place between the metal and the water present in the mold and more especially in the sand, and a similar reaction is then liable to take place between the metal and the molding material, such as sand, such reaction rendering the casting at least inferior in outer appearance. If great quantities of water are still present in the mold, explosion-like phenomena are even likely to occur.

In U. S. Patent No. 1463609 granted to Karl Gersbach, Oskar Hermann Weber and myself a method of casting is described which allows avoiding the ignition of the metal, provided that the molds are carefully dried, this method substantially consisting in dusting the mold with a material which will not react with the molten metal, either as such or in the form of its products of oxidation. I assume this protective effect to be due to the action of the gases or vapors developed from the protective material in contact with the hot metal and which prevent the access of air or steam to the metal.

I have now ascertained that by admixing certain materials to the sand or other material from which the mold is prepared for casting, I obtain the surprising result that the drying of the mold and of the sand or the like contained therein is no more necessary, the presence of moisture being innoxious so that I am now enabled to cast the metals in question in undried molds made of green sand. These materials (which may be called protective substances) are those described in the specification above cited, as being adapted to prevent oxidation of the castings when intensely dried molding sand

is used, and more especially sulphur. The peculiar action of the protective substances has not yet been cleared up completely. It seems that the steam and air are sufficiently diluted with gases or vapors produced from these substances or that they prevent in some other way the access of water vapor to the hot metal so that no visible action of the steam upon the metal occurs. However, I wish it to be understood that this is merely an attempt to explain the peculiar action of the protective substances.

If sulphur is employed as protective material and green sand as molding material, the quantity of sulphur must be proportionate to the thickness of the casting. An addition of 1-6% sulphur to the sand has proved advantageous, but I may employ up to 35%. By admixing the protective material with the sand a sound protective effect is obtained even at those places where the casting is comparatively thick such as gates, inasmuch as the protective gases or vapors are not developed merely on the surface of the mold, as in the case of superficial powdering or spraying on, but also from deeper layers in correspondence with the gradual heating of the mold by the metal as it flows in. However, in certain cases I may admix the protective material with the sand and besides powder or spray it onto the mold.

A similar effect within the scope of my invention might be obtained also by developing gases or vapors from the protective materials spoken of above out-side the mold and introducing them into the mold immediately before the casting. However, if this is done, the protective effect will be less powerful for the reason that the concentration of the protective masses or vapors will not be as great between the mold and the metal, as if they are generated in the mold itself.

The present application is divided out from patent of the United States No. 1584072 granted to me on May 11, 1926.

I wish it to be understood that I do not desire to be limited to the particular substances and modes of proceeding described, for obvious modifications will occur to a person skilled in the art.

I claim:

1. The method of making molds for casting easily oxidizable metals and alloys in undried molds, comprising preparing a mix-

ture of undried molding material and sulphur, and forming such mixture into a mold.

2. The method of making molds for casting easily oxidizable metals and alloys in undried molds, comprising preparing a mixture of undried molding material and 1% sulphur, and forming such mixture into a mold.

3. The method of making molds for casting easily oxidizable metals and alloys in undried molds, comprising preparing a mixture of undried molding material and more than 1%, but less than 35% sulphur, and forming such mixture into a mold. 10 15

In testimony whereof I affix my signature.

ADOLF BECK.